

W. FONDILLER.

METHOD OF MANUFACTURING INDUCTANCE COILS.

APPLICATION FILED SEPT. 12, 1914.

1,212,755.

Patented Jan. 16, 1917.



Witnesses:

*John G. Luttrell*

*O. E. Rasmussen*

Inventor:

William Fondiller  
by *John S. Roberts*  
ATT'y.

# UNITED STATES PATENT OFFICE.

WILLIAM FONDILLER, OF NEW YORK, N. Y., ASSIGNEE, BY MESNE ASSIGNMENTS, TO  
WESTERN ELECTRIC COMPANY, INCORPORATED, A CORPORATION OF NEW YORK.

## METHOD OF MANUFACTURING INDUCTANCE-COILS.

1,212,755.

Specification of Letters Patent.

Patented Jan. 16, 1917.

Application filed September 12, 1914. Serial No. 861,400.

To all whom it may concern:

Be it known that I, WILLIAM FONDILLER, a citizen of the United States, residing at New York, in the county of New York and State of New York, have invented certain new and useful Improvements in Methods of Manufacturing Inductance-Coils, of which the following is a full, clear, concise, and exact description.

10 This invention relates to inductance coils, such as loading coils, for telephone lines, and its object is to maintain constant the inductances of the line windings during the process of manufacture of the coils.

15 The usual steps in the manufacture of a loading coil are as follows: A very fine hard drawn iron wire is given a thin coating or film of insulating material and wound into a toroidal core, or the core may be formed of unannealed iron plates similarly coated.

20 The core is then insulated and insulated copper wire wound thereon, usually in sections. In the case of a phantom loading coil having air-gaps in its core, to which this invention is especially applicable, the copper wire is placed in inner and outer windings on a plurality of core sections, say four, the inner winding on one quarter section being connected in series with the outer winding

25 on the opposite quarter section. These two sectional windings together constitute one of the line windings of the phantom system. After the inner sectional windings are placed on the core, they are tested, compared and adjusted to a measured standard and compared one with the other, in order to insure that they will offer the same inductances to the telephonic currents. This is of the highest importance in order to meet

30 the close balance requirements for a phantom loading coil. Then the outer sectional windings are placed over the inner windings and tested and adjusted in a similar manner. The wound coils are then baked, preferably

35 in a vacuum, in order to drive out the moisture from the insulation on the copper wires, and immediately immersed in insulating compound which thoroughly impregnates the windings. Finally, after the coils are

40 taken out of this bath of insulating material and cooled, they are placed in protecting cases and sealed by filling the cases with an insulating compound. It has been found in following this process that changes in the

45 inductances of the windings occur by reason

50 of the heating of the coil core in the baking ovens and in the hot insulating compound, so that the careful testing and adjustment of the winding inductances were of little or no use. Furthermore, after the baking and the 55 impregnating of the wound coils, it is impossible then to make any readjustment of the inner sectional windings without wholly removing the outer layers. The tearing down of the coil, in order to add to or remove 60 turns from the inner windings, is objectionable because of high labor cost and loss due to the destruction of the outer windings.

65 It is of importance to obtain a stable magnetic condition of the core, more especially in phantom loading coils having air-gaps, because the proper fulfilment of the requirements for such coils necessitates the observance of a definite ratio of turns in the inner and outer sectional windings. Failure 70 to observe this ratio of turns would result in an increased effective resistance to the side-circuit connection of the phantom coil, and would also result in crosstalk between the 75 sides of the phantom circuit. It is highly 80 desirable, therefore, that the inductances of the several winding sections of the finished loading coil shall be the same as the fixed and measured value for which these winding sections were designed. Investigation 85 of the difficulty in manufacture referred to led to the discovery that the changes in inductance of the windings occurred by reason of a change in the initial permeability 90 of the material of the core, due to the heating of the core when the coil is in the baking oven or when it is immersed in the hot insulating compound. That is to say, the core material undergoes a molecular change 95 in the nature of annealing which materially alters the inductances of the windings.

100 According to this invention, the difficulty referred to is wholly avoided by subjecting the material of the core to a preliminary baking temperature, which is not exceeded by the subsequent steps in the process of manufacture. It is preferable also that the preliminary baking temperature be not any greater than the maximum temperature to 105 which the core is subsequently subjected, this in order that the hysteresis and eddy current losses in the iron core may not be increased more than absolutely necessary. These losses, it is noted, increase rapidly 110 with increase of permeability of the iron,

and in loading coils it is very essential that they be as small as possible.

In the accompanying drawing is shown in cross-section a loading coil and its inclosing case to assist in an understanding of the invention.

The core 1 of the loading coil is best made up of unannealed iron, and preferably of fine hard drawn iron wire wound in such a way as to form a ring or toroid. Preferably the core is cut at diametrically opposite points so that it becomes a discontinuous toroidal core of two sections separated by air-gaps. The drawing illustrates a phantom loading coil having windings 2 to 9 inclusive, windings 2 to 5 being the inner sectional windings, and 6 to 9 the outer ones. The preliminary baking of the core material is preferably done before the wire is formed into a core and before it is given a thin coating or film of insulation—this to avoid the probability of injury to the insulation. After the core wire is thus baked, insulated and formed into a toroidal core, the windings are placed on the core and the two gaps cut in the core between adjacent windings. The inner sectional windings are tested and adjusted before the outer sectional windings are placed over them, and then the outer windings are placed over the inner ones and tested and adjusted, all in the manner previously stated. The coil is then baked and dipped in insulating material. The temperature reached by the core in baking and while immersed in the insulating material should not materially exceed and preferably should be as nearly equal as possible to the preliminary core baking temperature. Finally, the coil is inserted in a protecting case 10 and insulating material 11 poured in, in the manner previously stated. The core temperature reached during this latter step should also be not greater than the preliminary core baking temperature.

It has been demonstrated that the subsequent heatings of the core in the baking oven and when the coil is dipped in the insulating compounds, does not materially change the initial permeability of the core provided the preliminary core baking temperature is not exceeded. In fact, any reasonable number of such limited heating operations may take place without materially changing the core characteristics, and therefore without altering the winding inductances from the fixed and measured value with which they had been compared.

What is claimed is:

1. The method of manufacturing induct-

tance coils which consists in subjecting the core material to a baking temperature, assembling the said material into a core, placing windings on the core, and subsequently heating the coil at a temperature approximately the same as the preliminary baking temperature.

2. The method of manufacturing inductance coils which consists in subjecting the core material to a baking temperature, placing windings on the core, baking the coil, and impregnating the coil in insulating compound, the maximum temperature of the core during the baking and impregnating steps being approximately the same as the preliminary core baking temperature. 75

3. The method of manufacturing inductance coils which consists in subjecting the core material to a baking temperature, placing a plurality of line winding sections on the core, comparing the inductances of the line winding sections with a standard inductance, and heating the coil at a temperature approximately the same as the preliminary core-baking temperature. 80

4. The method of manufacturing inductance coils which consists in subjecting the core material to a baking temperature, coating the said material with an insulating film, assembling the said material into a core, placing windings on the core, and heating the coil at a temperature approximately the same as the preliminary core-baking temperature. 85 90

5. The method of manufacturing inductance coils which consists in subjecting hard drawn iron wire to a baking temperature, forming the wire into a core, winding the core with insulated wire and heating the coil at a temperature approximately the same as the preliminary core wire baking 95 100 temperature.

6. The method of manufacturing cores for inductance coils which consists in subjecting hard drawn iron wire to a baking temperature, coating said wire with an insulating film and forming said coated wire into a core, the said wire baking temperature being substantially the same as the highest temperature to which the core is subsequently subjected in completing the 110 manufacture of the coil.

In witness whereof, I hereunto subscribe my name this 11 day of September A. D., 1914.

WILLIAM FONDILLER.

Witnesses:

ALICE HAZLEY,  
NANSA E. TUTHILL.